

G. W. BILLINGS.

Cleaning Fibres.

No. 41,826.

Patented March 8, 1864.

Fig. 1.



Witnesses;

J. H. Bullock  
C. Jones

Inventor;

G. W. Billings

# UNITED STATES PATENT OFFICE.

GEORGE W. BILLINGS, OF NEW YORK, N. Y.

## IMPROVEMENT IN CLEANING AND SEPARATING THE FIBERS OF FLAX AND HEMP.

Specification forming part of Letters Patent No. 41,826, dated March 8, 1864; antedated February 21, 1864.

*To all whom it may concern:*

Be it known that I, GEORGE W. BILLINGS, of the city, county, and State of New York, have discovered and invented a new and useful Method of Cleansing and Refining Flax and Hemp; and I do hereby declare that the following is a full and exact description thereof, reference being had to the accompanying drawings, and to the letters marked thereon, making a part of this specification.

The nature of my invention consists in removing from the fibers of flax and hemp, or any other fibrous substances of like or analogous character, all the silex, resin, and other foreign and deleterious matters, leaving the fiber perfectly free and clean, in condition ready to be worked by the ordinary or modern and improved machinery into any desired fabric.

Before being operated upon the fiber should be rotted and dressed clean and free from stones or wood. It may be rotted by water or dew; but I prefer that which has been rotted and dressed by my improved process and machinery.

Having constructed a vat or tank of any suitable size and material—say twenty feet long, four feet wide, and three feet deep—of seasoned hard pine, or of any hard wood or suitable material, I place in it a perforated platform raised two and one-half inches from the bottom for the purpose of forming a space between the fiber and bottom of the vat or tank to receive the deposits loosened and deposited from the fiber. I then place in the vat or tank, upon the perforated platform, the flax or hemp or other fiber in any way and form most convenient for handling, until it is filled to within eight inches of the top, upon which I place a lattice covering of any suitable wood of sufficient strength and weight to prevent the fiber from rising to the top of the vat or tank.

I then let into the vat or tank tepid water until it has covered the fiber to the depth of two or more inches, keeping it always covering the fiber, and at a temperature of near 90° Fahrenheit, by any of the known or usual artificial means. If the fiber is in proper condition when placed in the vat or tank in from ten (10) to fifteen (15) hours after the vat or tank is filled with the water, fermentation will

begin and continue from four (4) to six (6) days, by which time the separation and loosening of the silex, resin, and other foreign and deleterious matters is complete and the fermentation stops.

Should the condition of the fiber be such as to require a longer time, the fermentation will continue longer than the time I have specified, and the fiber must be left undisturbed until the fermentation ceases, which done I draw off the liquid from the vat or tank and rinse off the fiber before removing by forcing through it clean tepid water.

I then take the fiber from the vat or tank and thoroughly wash and dry it, which may be done by hand or by any suitable machinery. I prefer machinery, using steam in the following way and manner:

I construct a pipe or pipes of from three (3) to six (6) inches in diameter and about three (3) feet long, which I surround with a steam-jacket in such way as will enable me to introduce into the jacket superheated steam, and thereby raise the temperature inside the pipes to about four hundred (400) degrees Fahrenheit. The ends of the pipes are so arranged that after being filled with the fiber they can be readily and tightly closed. The pipes being filled with the fiber, by means of connecting-pipes I inject hot water or steam under a pressure of about seventy (70) pounds to the square inch into them from each end alternately, which forces from and carries away from the fiber all the silex, resin, and other foreign and deleterious matters which may still have remained with it when put into the pipes, the water or steam being ejected through the pipes until the fiber has been thoroughly cleaned. After the fiber is thus washed I introduce superheated steam into the steam-jacket, by which the fiber is thoroughly dried, after which it is taken from the pipes.

The pipes for washing may be made in nests of two or more and be operated by mechanical means, and the steam and hot water fed to them in the same way and manner, or any similar way and manner, that steam is applied to an engine. To accelerate the washing, alkali or soap may be added to the water.

I do not confine myself to the method above described of leaving the fiber in the vat or tank immersed in the same tepid water with

which the vat is first filled until it is removed to be washed and cleansed, but the tepid water may be changed as often as desired, the fiber continued to be immersed so long as fermentation continues, and to be removed for washing only and so soon as the fermentation ceases.

Figure 1 represents a cross-section of the wash and dry pipe and steam jacket.

*a* is the pipe to contain the fiber or material to be washed and dried; *b b*, the steam-jacket; *c c*, the pipes to supply the steam and water; *d d*, the ends of the pipe which are movable; *e*, the pipe through which the superheated steam is conveyed into the steam-jacket.

Having thus described my invention, what I claim, and desire to secure by Letters Patent, is—

The loosening and dissolving of all resinous matters, silex, and other foreign and deleterious substances from flax, hemp, and other fibrous substances of like or analogous character by fermentation and removing the same by washing and the moisture by drying, substantially as described and set forth.

GEO. W. BILLINGS.

Witnesses:

JOHN A. HILLERY,  
E. D. MOORE.